

# UNITED STATES PATENT OFFICE.

WILLIAM A. McADAMS, OF BAY SHORE, NEW YORK.

## ALUMINUM ALLOY AND METHOD OF PRODUCING THE SAME.

1,121,267.

Specification of Letters Patent. Patented Dec. 15, 1914.

No Drawing.

Application filed April 15, 1914. Serial No. 832,049.

*To all whom it may concern:*

Be it known that I, WILLIAM A. McADAMS, a citizen of the United States, and resident of Bay Shore, in the county of Suffolk and State of New York, have invented a new and useful Improvement in Aluminum Alloys and Methods of Producing the Same, of which the following is a specification.

My invention consists in an aluminum alloy and in the method of producing the same, with the object in view of providing an inexpensive alloy suitable for casting purposes, which will be very strong.

The alloy is composed of aluminum, copper, zinc and antimony, in which the amount of zinc exceeds the amount of antimony, the amount of copper exceeds the amount of zinc, and the amount of aluminum exceeds the amount of copper. The aforesaid elements are preferably combined in the following proportions, by weight: aluminum, one hundred parts; copper, eighteen parts; zinc, five parts, and antimony, three parts.

In producing the alloy, the method which I have found to be the best is as follows: About one-third of the aluminum is melted and raised to a high temperature. The copper is then introduced into the aluminum. The antimony is then introduced and the mass thoroughly agitated. The balance of the aluminum is then added to the mass and the temperature of the mass is then lowered and kept at a dull red heat. The zinc is then added to the mass and the mass agitated thoroughly to insure the proper mixing of the different metals. The composition will then be ready for casting at as low a temperature as possible and it should be reheated as little as possible for the casting operation.

The alloy, composed of the above materials combined in the proportions substantially as above set forth and by the method substantially as above set forth, will produce a very satisfactory casting metal in 45 which the articles cast from the metal will be very strong.

What I claim is:—

1. A composition of matter comprising aluminum, copper, zinc and antimony, in 50 which the amount of zinc exceeds the amount of antimony, the amount of copper exceeds the amount of zinc, and the amount of aluminum exceeds the amount of copper.

2. A composition of matter comprising 55 aluminum, copper, zinc and antimony, combined in substantially the following proportions, by weight: aluminum, one hundred parts; copper, eighteen parts; zinc, five parts; and antimony three parts. 60

3. The method of producing a composition of matter composed of aluminum, copper, zinc and antimony, consisting in melting a portion of the aluminum and raising it to a high temperature, introducing the 65 copper, introducing the antimony and the balance of the aluminum, then lowering the temperature of the mass and introducing the zinc, and thoroughly agitating the mass. 70

In testimony, that I claim the foregoing 70 as my invention, I have signed my name in presence of two witnesses, this 14th day of April, 1914.

WILLIAM A. McADAMS.

Witnesses:

F. GEORGE BARRY,  
LIDA M. EGBERT.